



US009303360B2

(12) **United States Patent**  
**Castro et al.**

(10) **Patent No.:** **US 9,303,360 B2**  
(b4) **Date of Patent:** **\*Apr. 5, 2016**

(54) **USE OF NANOCRYSTALINE CELLULOSE AND POLYMER GRAFTED NANOCRYSTALINE CELLULOSE FOR INCREASING RETENTION IN PAPERMAKING PROCESS**

(71) **Applicant:** **Ecolab USA Inc.**, Naperville, IL (US)

(72) **Inventors:** **David A. Castro**, DeKalb, IL (US); **Rangarani Karnati**, Naperville, IL (US); **Shawnee M. Wilson**, Downers Grove, IL (US); **Weiguo Cheng**, Naperville, IL (US); **Mei Liu**, Plainfield, IL (US); **Zhiyi Zhang**, Naperville, IL (US)

(73) **Assignee:** **ECOLAB USA Inc.**, St. Paul, MN (US)

(\*) **Notice:** Subject to any disclaimer, the term of this patent is extended or adjusted under 35 U.S.C. 154(b) by 0 days.

This patent is subject to a terminal disclaimer.

(21) **Appl. No.:** **13/962,569**

(22) **Filed:** **Aug. 8, 2013**

(65) **Prior Publication Data**

US 2015/0041089 A1 Feb. 12, 2015

(51) **Int. Cl.**

**D21H 21/10** (2006.01)  
**D21H 17/00** (2006.01)  
**D21H 17/25** (2006.01)  
**D21H 19/52** (2006.01)

(52) **U.S. Cl.**

CPC ..... **D21H 21/10** (2013.01); **D21H 17/25** (2013.01); **D21H 19/52** (2013.01)

(58) **Field of Classification Search**

USPC ..... 162/158, 164.1–164.7, 168.1–168.3,

162/168.7, 185, 175–178; 524/9, 13, 524/35–46; 435/277; 977/895–897

See application file for complete search history.

(56)

**References Cited**

**U.S. PATENT DOCUMENTS**

|               |         |                      |
|---------------|---------|----------------------|
| 2,178,139 A   | 10/1939 | Epstein et al.       |
| 2,202,601 A   | 5/1940  | Ried                 |
| 3,793,299 A * | 2/1974  | Zimmerer .....       |
| 4,374,702 A * | 2/1983  | Turbak .....         |
|               |         | D01D 5/11<br>162/100 |
| 4,385,961 A   | 5/1983  | Svending et al.      |
| 4,388,150 A   | 6/1983  | Sunden et al.        |
| 4,753,710 A   | 6/1988  | Langley et al.       |
| 4,783,314 A   | 11/1988 | Hoots et al.         |
| 4,913,775 A   | 4/1990  | Langley et al.       |

(Continued)

**FOREIGN PATENT DOCUMENTS**

|    |             |         |
|----|-------------|---------|
| WO | 2010-125247 | 11/2010 |
| WO | 2010-134868 | 11/2010 |

(Continued)

**OTHER PUBLICATIONS**

Smook, Gary A., Handbook for Pulp and Paper Technologists, 2nd ed, Angus Wilde Publications, 1992, pp. 224-225.\*

(Continued)

*Primary Examiner* — Dennis Cordray

(74) **Attorney, Agent, or Firm:** Eric D. Babych; Brinks Gilson & Lione

(57) **ABSTRACT**

The invention provides methods and compositions for improving the characteristics of paper substrates. The method involves adding to a paper substrate an NCC-polymer. NCC polymers have unique chemical properties which result in improvements in wet strength, dry strength and drainage retention properties of the paper substrates.

**12 Claims, 1 Drawing Sheet**



NCC

AA

AM

NCC/AM/AA copolymer

| (56)                                                    | References Cited |                               |                   |         |                                      |
|---------------------------------------------------------|------------------|-------------------------------|-------------------|---------|--------------------------------------|
| U.S. PATENT DOCUMENTS                                   |                  |                               |                   |         |                                      |
| 4,966,652 A                                             | 10/1990          | Wasser                        | 8,247,593 B2      | 8/2012  | Morrison et al.                      |
| 4,992,380 A                                             | 2/1991           | Moriarty et al.               | 8,247,597 B2      | 8/2012  | Fair et al.                          |
| 5,098,520 A                                             | 3/1992           | Begala                        | 8,258,208 B2      | 9/2012  | Kurian et al.                        |
| 5,167,776 A                                             | 12/1992          | Bhaskar et al.                | 8,262,852 B2      | 9/2012  | Duggirala et al.                     |
| 5,171,450 A                                             | 12/1992          | Hoots                         | 8,262,858 B2      | 9/2012  | Duggirala et al.                     |
| 5,182,062 A                                             | 1/1993           | Lee et al.                    | 8,288,835 B2      | 10/2012 | Quevy et al.                         |
| 5,254,221 A                                             | 10/1993          | Lowry et al.                  | 8,298,439 B2      | 10/2012 | Blubaugh et al.                      |
| 5,274,055 A                                             | 12/1993          | Honig et al.                  | 8,298,508 B2      | 10/2012 | Wang et al.                          |
| 5,346,589 A *                                           | 9/1994           | Braunstein et al. .... 162/72 | 8,302,778 B2      | 11/2012 | Tran                                 |
| 5,840,158 A                                             | 11/1998          | Choo et al.                   | 8,366,877 B2      | 2/2013  | Duggirala et al.                     |
| 6,071,379 A                                             | 6/2000           | Wong Shing et al.             | 8,382,947 B2      | 2/2013  | Skaggs et al.                        |
| 6,361,652 B2                                            | 3/2002           | Keiser et al.                 | 8,382,950 B2      | 2/2013  | Cheng                                |
| 6,361,653 B2                                            | 3/2002           | Keiser et al.                 | 8,398,901 B2      | 3/2013  | Beck et al.                          |
| 6,372,805 B1                                            | 4/2002           | Keiser et al.                 | 8,414,739 B2      | 4/2013  | Kimura et al.                        |
| 6,379,753 B1 *                                          | 4/2002           | Soane et al. .... 427/434.2   | 8,440,052 B2      | 5/2013  | Duggirala et al.                     |
| 6,486,216 B1                                            | 11/2002          | Keiser et al.                 | 8,444,812 B2      | 5/2013  | Grigoriev et al.                     |
| 6,592,718 B1                                            | 7/2003           | Wong Shing et al.             | 8,465,623 B2      | 6/2013  | Zhao et al.                          |
| 6,605,674 B1                                            | 8/2003           | Whipple et al.                | 8,945,345 B2 *    | 2/2015  | Laine ..... D21C 9/00<br>162/175     |
| 7,125,469 B2                                            | 10/2006          | Barcus et al.                 | 9,034,145 B2 *    | 5/2015  | Castro et al. .... 162/146           |
| 7,473,334 B2                                            | 1/2009           | Wong Shing et al.             | 2005/0025659 A1   | 2/2005  | Godfrey et al.                       |
| 7,497,924 B2 *                                          | 3/2009           | Nguyen et al. .... 162/157.6  | 2011/0182990 A1   | 7/2011  | Su et al.                            |
| 7,615,135 B2                                            | 11/2009          | Harrington et al.             | 2011/0196094 A1   | 8/2011  | Hamad et al.                         |
| 7,641,776 B2                                            | 1/2010           | Nagar et al.                  | 2011/0250341 A1   | 10/2011 | Keiser et al.                        |
| 7,829,738 B1                                            | 11/2010          | Brammer, Jr. et al.           | 2011/0277947 A1   | 11/2011 | Hua et al.                           |
| 7,995,504 B2                                            | 8/2011           | Ransom et al.                 | 2011/0293932 A1   | 12/2011 | Jiang et al.                         |
| 8,012,758 B2                                            | 9/2011           | Enzien et al.                 | 2013/0000855 A1 * | 1/2013  | Nuopponen ..... D21H 11/18<br>162/76 |
| 8,021,518 B2                                            | 9/2011           | Furman et al.                 | 2013/0139856 A1   | 6/2013  | Vinson et al.                        |
| 8,066,847 B2                                            | 11/2011          | Grigoriev et al.              | 2013/0146099 A1   | 6/2013  | Monsrud et al.                       |
| 8,067,629 B2                                            | 11/2011          | Tong                          | 2013/0146102 A1   | 6/2013  | Monsrud et al.                       |
| 8,071,667 B2                                            | 12/2011          | Furman, Jr. et al.            | 2013/0146425 A1   | 6/2013  | Tokhtuev                             |
| 8,082,649 B2                                            | 12/2011          | Rider                         | 2014/0083416 A1 * | 3/2014  | Nuopponen et al. .... 127/29         |
| 8,088,213 B2                                            | 1/2012           | Cheng et al.                  | WO 2010-1243785   | 11/2010 |                                      |
| 8,092,618 B2                                            | 1/2012           | Sharpe et al.                 | WO 2012-034997    | 3/2012  |                                      |
| 8,092,649 B2                                            | 1/2012           | Shevchenko et al.             |                   |         |                                      |
| 8,097,687 B2                                            | 1/2012           | Kurian et al.                 |                   |         |                                      |
| 8,101,045 B2                                            | 1/2012           | Furman et al.                 |                   |         |                                      |
| 8,123,042 B2                                            | 2/2012           | Tran                          |                   |         |                                      |
| 8,172,983 B2                                            | 5/2012           | Cheng et al.                  |                   |         |                                      |
| 8,242,287 B2                                            | 8/2012           | Schertzer et al.              |                   |         |                                      |
| 8,246,780 B2                                            | 8/2012           | Duggirala et al.              |                   |         |                                      |
| FOREIGN PATENT DOCUMENTS                                |                  |                               |                   |         |                                      |
|                                                         | WO               |                               |                   |         |                                      |
|                                                         | WO               |                               |                   |         |                                      |
| OTHER PUBLICATIONS                                      |                  |                               |                   |         |                                      |
| J. Peel, Paper Science & Paper Manufacture 1999, p. 90. |                  |                               |                   |         |                                      |
| * cited by examiner                                     |                  |                               |                   |         |                                      |



## 1

**USE OF NANOCRYSTALINE CELLULOSE  
AND POLYMER GRAFTED  
NANOCRYSTALINE CELLULOSE FOR  
INCREASING RETENTION IN  
PAPERMAKING PROCESS**

CROSS REFERENCE TO RELATED  
APPLICATIONS

Not Applicable.

STATEMENT REGARDING FEDERALLY  
SPONSORED RESEARCH OR DEVELOPMENT

Not Applicable.

BACKGROUND OF THE INVENTION

The invention relates to compositions, methods, and apparatuses for improving drainage retention, wet strength, and dry strength of paper in a papermaking process. A typical papermaking process includes the steps of: 1) pulping wood or some other source of papermaking fibers; 2) producing a paper mat from the pulp, the paper mat being an aqueous slurry of cellulosic fiber which may also contain additives such as inorganic mineral fillers or pigments; 3) depositing this slurry on a moving papermaking wire or fabric; 4) forming a sheet from the solid components of the shiny by draining the water; 5) pressing and drying the sheet to further remove water, and 6) potentially rewetting the dry sheet by passing it through a size press and further drying it to form a paper product.

When conducting a papermaking process, a number of concerns need to be taken into account to assure the quality of the resulting paper product. For example when draining water from the slurry, as many fibers and chemical additives should be retained and not flow out with the water. Similarly the resulting sheet should have adequate wet strength and dry strength.

As described for example in U.S. Pat. Nos. 7,473,334, 6,605,674, 6,071,379, 5,254,221, 6,592,718, 5,167,776 and 5,274,055 a number of retention aids such as polymers flocculants, and silica based microparticles, may be added to the slurry to facilitate drainage retention. The retention aids function to retain solid matter within the slurry as water is drained out of the slurry. In addition to retaining fibers, the retention aid should also retain additives such as optical brighteners, fillers, and strength agents. The selection of such retention aids is complicated by the fact that they must both allow for the free drainage of water from the slurry and also must not interfere with or otherwise degrade the effectiveness of other additives present in the resulting paper product.

As described for example in U.S. Pat. Nos. 8,465,623, 7,125,469, 7,615,135 and 7,641,776 a number of materials function as effective dry strength agents. These agents can be added to the slurry to increase the strength properties of the resulting sheet. As with retention aids however they must both allow for the free drainage of water from the slurry and also must not interfere with or otherwise degrade the effectiveness of other additives present in the resulting paper product.

As described for example in U.S. Pat. Nos. 8,414,739 and 8,382,947, surface strength agents are materials which increase the resistance of the resulting paper product to abrasive forces. Surface strength agents are often applied as coatings over the formed paper sheet at the size press. Of particular importance is that such agents be compatible with other items present in coatings such as sizing agents and optical

## 2

brightening agents. In addition desirable surface strength agents must not unduly impair the flexibility of the resulting paper product.

As it is difficult to increase dry strength, surface strength, and/or drainage retention while simultaneously not inhibiting other attributes of the paper or additives therein, there is an ongoing need for improved methods of improving dry strength, surface strength, and/or drainage retention. The art described in this section is not intended to constitute an admission that any patent, publication or other information referred to herein is "prior art" with respect to this invention, unless specifically designated as such. In addition, this section should not be construed to mean that a search has been made or that no other pertinent information as defined in 37 CFR §1.56(a) exists.

BRIEF SUMMARY OF THE INVENTION

To satisfy the long-felt but unsolved needs identified above, at least one embodiment of the invention is directed towards a method of improving a paper substrate used in a papermaking process. The method comprises the steps of: providing an NCC-polymer, and adding the NCC-polymer to a paper substrate in the wet end of a papermaking process, wherein the NCC-polymer is substantially distributed throughout the paper substrate.

The NCC-polymer may comprise a polymer chain bonded to an NCC core and the polymer chain is made up of one or more monomers selected from the list consisting of: vinyl acetate, acrylic acid, sodium acrylate, ammonium acrylate, methyl acrylate, acrylamide, acrylonitrile, N,N-dimethyl acrylamide, 2-acrylamido 2-methylpropane-1-sulfonic acid, sodium 2-acrylamido-2-methylpropane-1-sulfonate, 3-acrylamidopropyl-trimethyl-ammonium chloride, diallyldimethylammonium chloride, 2-(dimethylamino)ethyl acrylate, 2-(acryloyloxy)-N,N,N-trimethyllethanaminium chloride, N,N-dimethylaminoethyl acrylate benzyl chloride quaternary salt, 2-(acryloyloxy)-N,N,N-trimethyllethanaminium methyl sulfate, 2-(dimethylamino)ethyl methacrylate, 2-(methacryloyloxy)-N,N,N-trimethyllethanaminium chloride, 3-(dimethylamino)propyl methacrylamide, 2-(methacryloyloxy)-N,N,N-trimethyllethanaminium methyl sulfate, methacrylic acid, methacrylic anhydride, methyl methacrylate, methacryloyloxy ethyl trimethyl ammonium chloride, 3-methacrylamidopropyl-trimethyl-ammonium chloride, hexadecyl methacrylate, octadecyl methacrylate, docosyl acrylate, n-vinyl pyrrolidone, 2-vinyl pyridine, 4-vinyl pyridine, epichlorohydrin, n-vinyl formamide, acetamide, 2-hydroxyethyl acrylate glycidyl methacrylate, 3-(allyloxy)-2-hydroxypropane-1-sulfonate, 2-(allyloxy)ethanol, ethylene oxide, propylene oxide, 2,3-epoxypropyltrimethylammonium chloride, (3-glycidoxypropyl)trimethoxy silane, epichlorohydrin-dimethylamine, vinyl sulfonic acid sodium salt, sodium 4-styrene sulfonate, caprolactam and any combination thereof.

The NCC-polymer may be a graft polymer having at least two NCC cores linked at least in part by polymer chains. The NCC-polymer may be a branched polymer having a first polymer chain extending from an NCC core and at least one branch diverting away from the first polymer chain. At least one branch may be constructed out of a different selection of monomers than the first polymer chain, the different selection being different in monomer type, monomer ratio, or both. The NCC-polymer may increase the wet strength of the paper substrate. The NCC-polymer may increase the retention of solids during the drainage of liquid medium from the paper substrate.

Additional features and advantages are described herein, and will be apparent from, the following Detailed Description.

#### BRIEF DESCRIPTION OF THE DRAWINGS

A detailed description of the invention is hereafter described with specific reference being made to the drawings in which:

FIG. 1 is an illustration of a reaction forming an NCC/AM/AA polyelectrolyte copolymer.

For the purposes of this disclosure, like reference numerals in the figures shall refer to like features unless otherwise indicated. The drawings are only an exemplification of the principles of the invention and are not intended to limit the invention to the particular embodiments illustrated.

#### DETAILED DESCRIPTION OF THE INVENTION

The following definitions are provided to determine how terms used in this application, and in particular how the claims, are to be construed. The organization of the definitions is for convenience only and is not intended to limit any of the definitions to any particular category.

“Wet End” means that portion of the papermaking process prior to a press section where a liquid medium such as water typically comprises more than 45% of the mass of the substrate, additives added in a wet end typically penetrate and distribute within the slurry.

“Dry End” means that portion of the papermaking process including and subsequent to a press section where a liquid medium such as water typically comprises less than 45% of the mass of the substrate, dry end includes but is not limited to the size press portion of a papermaking process, additives added in a dry end typically remain in a distinct coating layer outside of the slurry.

“Consisting Essentially of” means that the methods and compositions may include additional steps, components, ingredients or the like, but only if the additional steps, components and/or ingredients do not materially alter the basic and novel characteristics of the claimed methods and compositions.

“Flocculant” means a composition of matter which when added to a liquid carrier phase within which certain particles are thermodynamically inclined to disperse, induces aggregations of those particles to form as a result of weak physical forces such as surface tension and adsorption, flocculation often involves the formation of discrete globules of particles aggregated together with films of liquid carrier interposed between the aggregated globules, as used herein flocculation includes those descriptions recited in ASTME 20-85 as well as those recited in Kirk-Othmer Encyclopedia of Chemical Technology, 5th Edition, (2005), (Published by Wiley, John & Sons, Inc.).

“Surface Strength” means the tendency of a paper substrate to resist damage due to abrasive force.

“Dry Strength” means the tendency of a paper substrate to resist damage due to shear force(s), it includes but is not limited to surface strength.

“Wet Strength” means the tendency of a paper substrate to resist damage due to shear force(s) when rewet.

“Wet Web Strength” means the tendency of a paper substrate to resist shear force(s) while the substrate is still wet.

“Substrate” means a mass containing paper fibers going through or having gone through a papermaking process, substrates include wet web, paper mat, slurry, paper sheet, and paper products.

“Paper Product” means the end product of a papermaking process it includes but is not limited to writing paper, printer paper, tissue paper, cardboard, paperboard, and packaging paper.

5 “NCC” or “NCC Core” means nano-crystalline cellulose. NCC Core is a discrete mass of NCC crystal onto which polymers may be grafted. an NCC or NCC core may or may not have been formed by acid hydrolysis of cellulose fibers and NCC or NCC core may or may not have been modified by this hydrolysis to have functional groups appended thereto including but not limited to sulfate esters.

10 “NCC-Polymer” means a composition of matter comprising at least an NCC core with at least one polymer chain extending therefrom.

15 “NCC Coupling” means a composition of matter comprising at least two NCC cores, the coupling can be a polymer linkage in which at least in part a polymer chain connects the two NCC cores, or it can be an NCC twin in which two (or more) NCC cores are directly connected to each other by a sub polymer linkage (such as epoxide) and/or direct bonding of one or more of the NCC cores’ atoms.

20 “Consisting Essentially of” means that the methods and compositions may include additional steps, components, ingredients or the like, but only if the additional steps, components and/or ingredients do not materially alter the basic and novel characteristics of the claimed methods and compositions.

25 “Slurry” means a mixture comprising a liquid medium such as water within which solids such as fibers (such as cellulose fibers) and optionally fillers are dispersed or suspended such that between >99% to 45% by mass of the slurry is liquid medium.

30 “Surfactant” is a broad term which includes anionic, non-ionic, cationic, and zwitterionic surfactants. Enabling descriptions of surfactants are stated in *Kirk-Othmer, Encyclopedia of Chemical Technology*, Third Edition, volume 8, pages 900-912, and in *McCutcheon’s Emulsifiers and Detergents*, both of which are incorporated herein by reference.

35 “Size Press” means the part of the papermaking machine where the dry paper is rewet by applying a water-based formulation containing surface additives such as starch, sizing agents and optical brightening agents, a more detailed description of size press is described in the reference *Handbook for Pulp and Paper Technologists*, 3rd Edition, by Gary A. Smook, Angus Wilde Publications Inc., (2002).

40 In the event that the above definitions or a description stated elsewhere in this application is inconsistent with a meaning (explicit or implicit) which is commonly used, in a dictionary, or stated in a source incorporated by reference into this application, the application and the claim terms in particular are understood to be construed according to the definition or description in this application, and not according to the common definition, dictionary definition, or the definition 45 that was incorporated by reference. In light of the above, in the event that a term can only be understood if it is construed by a dictionary, if the term is defined by the Kirk-Othmer Encyclopedia of Chemical Technology, 5th Edition, (2005), (Published by Wiley, John Sons, Inc.) this definition shall control how the term is to be defined in the claims.

50 At least one embodiment of the invention is directed towards adding at least one NCC-Polymer to a paper substrate in a papermaking process. The NCC-Polymer may be added in the wet end and/or in the dry end. The NCC-Polymer may be added as a coating outside of the substrate or may be dispersed within the substrate. A coating may partially or fully enclose the substrate. The NCC-Polymer may comprise

linear, branched, cyclic, polymers extending from the NCC core and/or may be an NCC Graft Polymer.

As described in US Published Patent Applications 2011/0293932, 2011/0182990, 2011/0196094, and U.S. Pat. No. 8,398,901, NCC are naturally occurring crystals present in plant fibers. A typical cellulose bearing fiber comprises regions of amorphous cellulose and regions of crystalline cellulose. NCC can be obtained by separating the crystalline cellulose regions from the amorphous cellulose regions of a plant fiber. Because their compact nature makes crystalline cellulose regions highly resistant to acid hydrolysis, NCC is often obtained by acid hydrolyzing plant fibers. NCC crystallites may have 5-10 nm diameter and 100-500 nm length. NCC may have a crystalline fraction of no less than 80% and often between 85% and 97%.

NCC is an extremely strong material but its use as an additive in paper products is constrained because of its small size. As stated in US Published Patent Application 2011/0277947 ¶[0019], because NCC is an extremely short subset of a fiber, it does not have sufficient length to impart strength aiding qualities to the long stretches of paper fibers.

In at least one embodiment the composition added to a papermaking substrate comprises an NCC core with at least one polymer chain extending from the NCC core. NCC comprises a number of hydroxyl groups which are possible anchor sites from which polymer chains may extend. Without being limited by a particular theory or design of the invention or of the scope afforded in construing the claims, it is believed that because of its unique aspect ratio, density, anchor sites, rigidity and supporting strength, NCC-Polymers are able to arrange polymer chains in unique arrangements that afford a number of unique properties that enhance paper characteristics.

In at least one embodiment the NCC-Polymer is added in the wet end of a papermaking process. In at least one embodiment the NCC-Polymer is added as a coating in the size press of a papermaking process. Detailed descriptions of the wet and dry ends of a papermaking process and addition points for chemical additives therein are described in the reference *Handbook for Pulp and Paper Technologists, 3rd Edition*, by Gary A. Smook, Angus Wilde Publications Inc., (2002). The NCC-Polymer may be added to the papermaking process at any addition point(s) described therein for any other chemical additive and according to the methods and with any of the apparatuses also described therein.

In at least one embodiment the NCC-Polymer is formed by the derivatization of one or more hydroxyl groups on an NCC crystal through condensation polymerization or grafting of vinyl monomers via radical polymerization to meet desired end user requirements.

In at least one embodiment the polymer attached to the NCC core is a polysaccharide. In at least one embodiment the polysaccharide NCC-Polymer is used as viscosity modifier in enhanced oil recovery, as flocculants for wastewater treatment and filler strength agent in a papermaking process.

In at least one embodiment the polymer attached to the NCC core is a vinyl polymer. In at least one embodiment it is a copolymer having structural units of at least two vinyl monomers including but not limited to acrylamide and acrylic acid. Polyacrylamide, polyacrylic acid, and 2-(methacryloyloxy)ethyl trimethylammonium chloride are efficient flocculants for water treatment and various applications. However, vinyl polymers show limited biodegradability and poor shear stability whereas nanocrystalline cellulose (NCC) is shear stable but are less efficient as flocculants. Connecting non-

ionic, anionic, and/or cationic vinyl monomers on an NCC core yields better performing polyelectrolyte flocculants, and filler materials.

In at least one embodiment the NCC-polymer is added to the papermaking process alongside 2-(methacryloyloxy)ethyl trimethylammonium chloride. In at least one embodiment the NCC-polymer added to a papermaking process is exposed to shear in excess to what a non-NCC-polymer can endure and still function, and continues to function.

In at least one embodiment the NCC-polymer is a branched polymer in which from a first chain of polymer structural units extending from the NCC core, one or more distinct other chains branch off from the first polymer chain and/or from other distinct chain branches. In at least one embodiment the first chain is comprised of a different variety of monomer units than one or more of the branch chains. Differences in chain compositions allows for versatile polymer arrangements as a means of imparting a variety of functional groups to a polymer. It also permits one to combine the best properties of two or more polymers in one physical unit. For example the first chain may be selected for its capacity to support or position functionally active polymer branches according to a geometry which has superior effects.

In at least one embodiment the polymer chain/branch is grown according to one or more of: a grow-to method, a grow-from method, and/or a grow-through method. In the grow-to approach an end group of a pre-formed polymer is coupled with a functional group on the NCC core. In the growing-from approach, the growth of the polymer chain occurs from initiation sites attached to the NCC core. In the growing-through approach a vinyl macro-monomer of cellulose is copolymerized from the NCC core with low molecular weight co-monomer.

Representative examples of vinyl monomers which can be used for any of the three growth approaches include but are not limited to vinyl acetate, acrylic acid, sodium acrylate, ammonium acrylate, methyl acrylate, acrylamide, acrylonitrile, N,N-dimethyl acrylamide, 2-acrylamido-2-methylpropane-1-sulfonic acid, sodium 2-acrylamido-2-methylpropane-1-sulfonate, 3-acrylamidopropyl-trimethylammonium chloride, diallyldimethylammonium chloride, 2-(dimethylamino)ethyl acrylate, 2-(acryloyloxy)-N,N,N-trimethyl-ethanaminium chloride, N,N-dimethylaminoethyl acrylate benzyl chloride quaternary salt, 2-(acryloyloxy)-N,N,N-trimethyl-ethanaminium methyl sulfate, 2-(dimethylamino)ethyl methacrylate, 2-(methacryloyloxy)-N,N,N-trimethyl-ethanaminium chloride, 2-(methacryloyloxy)-N,N,N-trimethyl-ethanaminium methyl sulfate, 3-(dimethylamino)propyl methacrylamide, methacrylic acid, methacrylic anhydride methyl methacrylate, methacryloyloxy ethyl trimethyl ammonium chloride, 3-methacrylamidopropyl-trimethyl-ammonium chloride, hexadecyl methacrylate, octadecyl methacrylate, docosyl acrylate, n-vinyl pyrrolidone, 2-vinyl pyridine, 4-vinyl pyridine, epichlorohydrin, formamide, n-vinyl acetamide, 2-hydroxyethyl acrylate glycidyl methacrylate, 3-(allyloxy)-2-hydroxypropane-1-sulfonate, 2-(allyloxy)ethanol, ethylene oxide, propylene oxide, 2,3-epoxypropyltrimethylammonium chloride, (3-glycidoxypropyl)trimethoxy silane, epichlorohydrin-dimethylamine, vinyl sulfonic acid sodium salt, Sodium 4-styrene sulfonate, caprolactam and any combination thereof.

In at least one embodiment addition of an NCC-polymer to a papermaking furnish or slurry improves drainage retention. As shown in the Examples, NCC-polymers used alongside starch, a cationic flocculant and an acrylic acid polymer have superior retention performance to such drainage programs lacking the NCC-polymers. Improved retention of fines, fill-

ers, and other components of the furnish decreases the amount of such components lost to the whitewater and hence reduces the amount of material wastes, the cost of waste disposal and the adverse environmental effects. It is generally desirable to reduce the amount of material employed in a papermaking process.

In at least one embodiment adding NCC-polymer to a papermaking furnish or slurry improves wet strength. As described in U.S. Pat. No. 8,172,983, a high degree of wet strength in paper is desired to allow for the addition of more filler (such as PCC or GCC) to the paper. Increasing filler content results in superior optical properties and cost savings (filler is cheaper than fiber).

In at least one embodiment the NCC-polymer is added as a coating or as part of a coating during size press of a papermaking process. The NCC-polymer may be added as a coating applied during a size press operation and may be added alongside starch, sizing agents or any other additive added during the size press.

In at least one embodiment the NCC-polymer added to the papermaking process is an NCC graft polymer. The graft polymer comprises two or more NCC cores. The NCC graft polymer may include a single polymer chain bridging between the NCC cores. The NCC Graft may also include two or more NCC cores with distinct polymer chains that are cross-linked to each other. As such a NCC-polymer is cross-linked to at least one other NCC-polymer where the cross-linkage is located at one of the structural units of the polymer and not at the NCC core. The cross linkage may be achieved by one or more polymer crosslinking agents known in the art. The NCC graft polymer may be in the form of a hydrogel as described in US Published Patent Application 2011/0182990.

In at least one embodiment a composition is added to a commercial process. The composition is a mixture comprising: a) NCC mixed with a polymer additive that is not an NCC-polymer, b) NCC mixed with a polymer additive that is an NCC-polymer, and/or c) a polymer additive which is an NCC-Polymer. In at least one embodiment the polymer additive is a polymer made up of one or more of NCC, non-ionic, water-soluble monomers, anionic monomers, cationic monomers, and any combination thereof. The polymer additives may be manufactured according any process described in the references: Emulsion Polymerization and Emulsion Polymers, by Peter A. Lovell et al, John Wiley and Sons, (1997), Principles of polymerization, Fourth Edition, by George Odian, John Wiley and Sons, (2004), Handbook of RAFT Polymerization, by Christopher Barner-Kowollik, Wiley-VCH, (2008), Handbook of Radical Polymerization, by Krzysztof Matyjaszewski et al, John Wiley and Sons, (2002), Controlled/Living Radical Polymerization: Progress in ATRP, NMP, and RAFT: by K. Matyjaszewski, Oxford University Press (2000), and Progress in Controlled Radical Polymerization: Mechanisms and Techniques, by Krzysztof Matyjaszewski et al, ACS Symposium Series 1023 (2009). The polymer additives may be manufactured according any process including but not limited to Solution, emulsion, inverse-emulsion, dispersion, atom transfer radical polymerization (ATRP), Reversible addition-fragmentation-chain transfer polymerization (RAFT), and ring opening polymerization.

The polymer additive may be added to any known chemical feed point in any of commercial process such as:

Industrial wastewater treatment including: solids liquids separations in clarification, dissolved air flotation, induced air flotation, dewatering, and raw water treatment,

Oil separation applications. Filtration aids, metals removal.

Paper, paperboard, tissue, and pulp manufacture including: manufacture process improvement, fine particle retention and dewatering, coatings and surface treatments, functional additives

5 Cooling water treatment including: Calcium Carbonate inhibitor, Calcium phosphate inhibitor, Zinc phosphate stabilizer, Iron and/or silt dispersant, Biodispersant, Silica scale inhibitor, Scale inhibitor for other species (e.g. Calcium Fluoride, Calcium sulfate, etc etc), Dual corrosion and scale inhibitor

10 Oil well treatment fluids and their application including: Drilling fluids and operations, Cement and cementing operations, Completion fluids and operations, Stimulation fluids (Acidizing and Fracturing) and operations, Water conformance chemistries and applications, Also Enhanced Oil Recovery EOR) chemistries and operation

15 Industrial warewash applications including: Reduction in hardness of wash water; Prevention of hard water film accumulation; Inhibition of corrosion of metal wares; Soil removal from wares; Prevention of soil redeposition

20 Industrial laundry applications including: Reduction in hardness of wash water; Prevention of hard water film accumulation; Prevention of hard water encrustation of fabrics; Dewatering of fabric; Soil release from fabric; Prevention of soil accumulation on fabrics; Prevention of soil redeposition in wash; Color retention of fabrics; Prevention of dye transfer in wash; Delivery of softening agents to fabrics; Delivery of antimicrobial agents to fabrics; Delivery of fragrance to fabric

25 30 Healthcare applications including: Inhibition of corrosion of metal instruments during cleaning/processing

35 Mining and Mineral Processing including: Process additives applied in the mining or transporting of a mineral substrate, in any mineral beneficiation process or related waste treatment process. Mining and mineral processing includes but not limited to: alumina, coal, copper, precious metals and sand and gravel. Applications covered includes but not limited to: solid liquid separations, flotation, scale control, dust control, metals removal and crystal growth modifiers

40 Silica Materials and Process applications including: Binder for strength improvement, Slip and investment casting, Catalysts industry (template), Refractories, Abrasion and polishing, Antifoam, Printing (inkjet/offset), Drainage aids.

45 Any commercial process described in one or more of: U.S. patent application Ser. Nos. 13/416,272 and 13/730,087, US Published Patent Application 2005/0025659, 2011/0250341 A1, 2013/0146099, 2013/0146102, 2013/0146425, 2013/0139856, and/or U.S. Pat. Nos. 2,202,601, 2,178,139, 8,465, 623, 4,783,314, 4,992,380, 5,171,450, 6,486,216, 6,361,653, 5,840,158, 6,361,652, 6,372,805, 4,753,710, 4,913,775, 4,388,150, 4,385,961, 5,182,062, 5,098,520, 7,829,738, 8,262,858, 8,012,758, 8,288,835, 8,021,518, 8,298,439, 8,067,629, 8,298,508, 8,066,847, 8,298,439, 8,071,667, 8,302,778, 8,088,213, 8,366,877, 8,101,045, 8,382,950, 55 8,092,618, 8,440,052, 8,097,687, 8,444,812, 8,092,649, 8,465,623, 8,082,649, 8,101,045, 8,123,042, 8,242,287, 8,246,780, 8,247,593, 8,247,597, 8,258,208, and/or 8,262, 852.

60 Representative non-ionic, water-soluble monomers suitable for use in the polymer additive include one or more of: acrylamide, methacrylamide, N,N-dimethylacrylamide, N,N-diethylacrylamide, N-isopropylacrylamide, N-vinylformamide, N-vinylmethylacetamide, N-vinyl pyrrolidone, 2-vinyl pyridine, 4-vinyl pyridine, epichlorohydrin, acrylonitrile, hydroxyethyl methacrylate, hydroxyethyl acrylate, hydroxypropyl acrylate, hydroxypropyl methacrylate, hexadecyl methacrylate, octadecyl Methacrylate, glycidyl meth-

acrylate, 3-(glycidoxypropyl)trimethoxy silane, 2-allyloxy ethanol, docosyl acrylate, N-t-butylacrylamide, N-methylacrylamide, epichlorohydrin-dimethylamine, caprolactam, and the like.

Representative anionic monomers suitable for use in the polymer additive include one or more of: acrylic acid, and its salts, including, but not limited to sodium acrylate, and ammonium acrylate, methacrylic acid, and its salts, including, but not limited to sodium methacrylate, and ammonium methacrylate, 2-acrylamido-2methylpropanesulfonic acid (AMPS), the sodium salt of AMPS, sodium vinyl sulfonate, styrene sulfonate, maleic anhydride, maleic acid, and its salts, including, but not limited to the sodium salt, and ammonium salt, sulfonate itaconate, sulfopropyl acrylate or methacrylate, or other water-soluble forms of these or other polymerisable carboxylic or sulphonic acids and crotonic acid and salts thereof. Sulfomethylated acrylamide, allylsulfonate, sodium vinyl sulfonate, itaconic acid, acrylamidomethyl butanoic acid, fumaric acid, vinylphosphonic acid, vinylsulfonic acid, vinylsulfonic acid sodium salt, allylphosphonic acid, 3-(allyloxy)-2-hydroxypropane sulfonate, sulfomethylated acrylamide, phosphono-methylated acrylamide, ethylene oxide, propylene oxide and the like.

Representative cationic monomers suitable for use in the polymer additive include one or more of: dialkylaminoalkyl acrylates and methacrylates and their quaternary or acid salts, including, but not limited to, dimethylaminoethyl acrylate methyl chloride quaternary salt, dimethylaminoethyl acrylate methyl sulfate quaternary salt, dimethylaminoethyl acrylate benzyl chloride quaternary salt, dimethylaminoethyl acrylate sulfuric acid salt, dimethylaminoethyl acrylate hydrochloric acid salt, dimethylaminoethyl methacrylate methyl chloride quaternary salt, dimethylaminoethyl methacrylate methyl sulfate quaternary salt, dimethylaminoethyl methacrylate benzyl chloride quaternary salt, dimethylaminoethyl methacrylate sulfuric acid salt, dimethylaminoethyl methacrylate hydrochloric acid salt, dialkylaminoalkylacrylamides or methacrylamides and their quaternary or acid salts such as acrylamidopropyltrimethylammonium chloride, dimethylaminopropylacrylamide methyl sulfate quaternary salt, dimethylaminopropylacrylamide sulfuric acid salt, dimethylaminopropyl acrylamide hydrochloric acid salt, methacrylamide propyltrimethylammonium chloride, dimethylaminopropyl methacrylamide methyl sulfate quaternary salt, dimethylaminopropyl methacrylamide sulfuric acid salt, dimethylaminopropyl methacrylamide hydrochloric acid salt, diethylaminoethylacrylate, diethylaminoethylmethacrylate, diallyldiethylammonium chloride, diallyldimethyl ammonium chloride and 2,3-epoxypropyltrimethylammonium chloride. Alkyl groups are generally C1-4 alkyl.

## EXAMPLES

The foregoing may be better understood by reference to the following examples, which are presented for purposes of illustration and are not intended to limit the scope of the invention. In particular the examples demonstrate representative examples of principles innate to the invention and these principles are not strictly limited to the specific condition recited in these examples. As a result it should be understood that the invention encompasses various changes and modifications to the examples described herein and such changes and modifications can be made without departing from the spirit and scope of the invention and without diminishing its

intended advantages. It is therefore intended that such changes and modifications be covered by the appended claims.

5

### Example #1

A number of NCC-polymers were made according to a growing-from approach. A 4-neck, 1.5 L reactor was fitted with a) an overhead mechanical stirrer connected to a metal shaft and a conical stirrer, b) a nitrogen inlet and sparge tube, c) a claisen adapter fitted with a reflux condenser d) a temperature probe (RTD) inserted through Teflon connector and temperature was controlled by Athena. To the reactor was added a 562.5 mL of pH adjusted NCC ( $1.14 \times 10^{-6}$  mol, 2.81 g, pH=2) dispersion and purged with  $N_2$  for 30 min and then ceric ammonium nitrate (CAN,  $1.12 \times 10^{-3}$  mol, 6.17 g) was allowed to react with NCC backbone for 15 min under  $N_2$  at R.T. The reactor was set to 70° C. and then 52.41 g of acrylamide ( $7.38 \times 10^{-1}$  mol), 17.08 g of acrylic acid ( $3.16 \times 10^{-1}$  mol) and water (84.67 g) were added to reactor at 42° C. Reaction mixture was heated to 70° C. and was maintained at 70° C. for 6 h. At 45 min 160 ppm of sodium hypo phosphite was added. Reaction was monitored by HNMR analysis of reaction aliquots (quenched with 500-1000 ppm of hydroquinone) and reached 92% conversion in 6 h (Table 2). Post modification was carried out using potassium persulfate (KPS, 500  $\mu$ mol) and sodium metabisulfite (SBS, 3500  $\mu$ mol) to burn out residual monomers. The nitrogen sparge was maintained throughout the reaction. The final pH of polymer was adjusted to 3.5 with NaOH and submitted to application testing. All samples were submitted for residual acrylamide and acrylic acid analyses Results are shown in Table 1.

35

TABLE 1

| Anionic NCC-Polymers Sample data. |          |           |       |             |      |                 |     |
|-----------------------------------|----------|-----------|-------|-------------|------|-----------------|-----|
| 40                                | Sample   | Sample    | Mol % |             |      | Residuals (ppm) |     |
|                                   |          |           | Id    | Description | AA   | AM              |     |
|                                   | 6653-145 | NCC/AA/AM | 30    | 70          | 3.5  | 746             | 63  |
|                                   | 6653-157 | NCC/AA/AM | 70    | 30          | 3.5  | 566             | 352 |
|                                   | 6653-159 | NCC/AA/AM | 50    | 50          | 3.7  | 524             | 112 |
|                                   | 6653-179 | NCC/AA    | 100   | —           | 1.58 | 340             | —   |

45

Note:  
Total active solids: 8% for all polyelectrolytes

50 The NCC-polymers were then added to a paper furnish. The alkaline furnish had a pH of 8.1 and was composed of 80% by weight cellulosic fibers and 20% precipitate calcium carbonate diluted to a consistency of 0.5% by weight. The fiber consisted of 2/3 bleached hardwood kraft and 1/3 bleached softwood kraft. The retention performance of NCC and polymer-grafted NCC was evaluated using the Britt Jar test method. The testing sequence is shown below.

55

TABLE 2

|    |            |                                     |
|----|------------|-------------------------------------|
| 60 | t = 0 sec  | Start                               |
|    | t = 5 sec  | Starch @ 10.0 #/t                   |
|    | t = 20 sec | Flocculant                          |
|    | t = 55 sec | NCC-polymer or comparison additives |
| 65 | t = 60 sec | Drain                               |
|    | t = 90 sec | Stop                                |

## 11

500 ml of furnish was charged in Britt jar and mixed at 1250 rpm. Starch Solvitose N was then charged at 10 lb/ton dry weight at 5 seconds. Cationic flocculant 61067 was charged at 20 seconds. Then at 55 seconds, NCC or NCC-polymer was charged. Drain started at 60 seconds and ended at 90 seconds. The drain (filtrate) was collected for turbidity measurement. The turbidity of the filtrate is inversely proportional to the furnish retention performance. The turbidity reduction % is proportional to the retention performance of the retention program. The higher the turbidity reduction %, the higher the retention of lines/or fillers. Two commercially available products, Nalco 8677Plus polyacrylic acid polymer and Nalco 8699 (a silica product), were tested for retention performance as references.

## 12

(PCC) as filler. 18 lb/ton cationic starch Stalok 310 was added as conventional dry strength agent, and various doses of NCC, NCC-polymer and N-1044 were added after cationic starch. 1 lb/ton N-61067 was added as retention aid. The treated furnish was used to make handsheet using Noble & Wood handsheet mold. The paper was pressed using a static press and dried by passing it once through a drum dryer at about 105°C. The resulted handsheets were allowed to equilibrate at 23°C. and 50% relative humidity for at least 12 hours before testing. Five duplicate handsheets were made for each condition and the mean values were reported.

10 A summary of the handsheet results was listed in the table below.

TABLE 4

| Exp | Dry Strength | Dry Strength  | Basis Weight |     | Ash content |     | ZDT (kPa) |      |       |           | Tensile Index (N · m/g) |      |      |             |
|-----|--------------|---------------|--------------|-----|-------------|-----|-----------|------|-------|-----------|-------------------------|------|------|-------------|
|     |              |               | Mean         | σ   | Mean        | σ   | Mean      | σ    | Est.  | at 20% AC | Increase                | Mean | σ    | I at 20% AC |
| No. | Type         | Dose (lb/ton) |              |     |             |     |           |      |       |           |                         |      |      |             |
| 1   | None         | 0.0           | 75.7         | 0.7 | 19.5        | 0.7 | 366.8     | 16.7 | 362.3 | 0.0%      | 25.0                    | 1.2  | 24.6 | 0.0%        |
| 2   | None         | 0.0           | 77.8         | 0.6 | 25.2        | 0.4 | 312.0     | 22.6 | 362.3 | 0.0%      | 20.2                    | 1.6  | 24.6 | 0.0%        |
| 3   | 1044         | 2.0           | 74.9         | 0.5 | 18.5        | 0.3 | 426.0     | 20.0 | 411.5 | 13.6%     | 31.5                    | 1.4  | 30.2 | 22.8%       |
| 4   | 1044         | 4.0           | 74.5         | 0.8 | 17.2        | 0.5 | 479.4     | 13.3 | 452.1 | 24.8%     | 33.7                    | 0.9  | 31.3 | 27.1%       |
| 5   | NCC-polymer  | 2.0           | 74.4         | 0.4 | 18.1        | 0.4 | 460.2     | 16.3 | 441.9 | 22.0%     | 33.8                    | 1.9  | 32.2 | 30.7%       |
| 6   | NCC-polymer  | 4.0           | 72.8         | 0.4 | 15.9        | 0.4 | 488.8     | 16.8 | 449.3 | 24.0%     | 35.6                    | 1.5  | 32.1 | 30.4%       |
| 7   | NCC          | 2.0           | 77.8         | 0.3 | 20.3        | 0.4 | 367.8     | 8.8  | 370.5 | 2.3%      | 26.0                    | 0.8  | 26.3 | 2.7%        |
| 8   | NCC          | 4.0           | 77.7         | 0.5 | 20.5        | 0.4 | 352.1     | 17.3 | 356.6 | -1.6%     | 24.9                    | 0.6  | 25.3 | 3.0%        |

TABLE 3

| Turbidity reduction % of the filtrates from Britt jar test |       |                |            |        |           |  |
|------------------------------------------------------------|-------|----------------|------------|--------|-----------|--|
| Material                                                   | Blank | Nalco 8677Plus | Nalco 8699 | NCC AA | NCC/AM/AA |  |
| 0.00 lb/ton                                                | 41.9  |                |            |        |           |  |
| 0.125 lb/ton                                               |       |                | 66.6       |        |           |  |
| 0.25 lb/ton                                                |       |                |            | 70.5   | 61.9      |  |
| 0.5 lb/ton                                                 |       |                | 66.7       | 67.8   | 60.6      |  |
| 1.0 lb/ton                                                 | 56.5  | 45.8           | 70.9       | 66.9   | 58.7      |  |
| 2.0 lb/ton                                                 |       | 58.1           | 81.0       | 66.2   |           |  |

As seen from the data, at the tested dosage range of 0.5 lb/ton to 2.0 lb./ton, NCC provided additional 28.8% to 39.1% turbidity reduction in comparison to the blank example, which well-performed than the two references 8677Plus and 8699. Nalco 8677Plus at 1.0 lb./ton showed only 14.6% more turbidity reduction than the blank and Nalco 8699 at 2.0 lb./ton showed only 16.2% more turbidity reduction than the blank. NCC-polymer with acrylic acid (NCC/AA) and acrylamide/acrylic acid (NCC/AM/AA) showed 25% more turbidity reduction and 18% more turbidity reduction respectively than the blank. The results revealed that both NCC and NCC-Polymer significantly improve turbidity reduction of tested furnish, which can lead better retention efficiency and cost reduction in paper production.

## Example #2

The experiments contrasted the ability of NCC and NCC-polymer to increase sheet dry strength as comparison as a conventional polyacrylamide based dry strength agent N-1044. NCC-polymer used in this example is 6653-1.45 listed in Table 1. The furnish contained 60% hardwood and 20% softwood and 20% precipitated calcium carbonate

35 50 40 45 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830

TABLE 5

| Condition | Starch, lb/t | AA/AM, lb/t | NCC, lb/t | Abrasion loss, mg/1000 revs |
|-----------|--------------|-------------|-----------|-----------------------------|
| 1         | 20.2         | —           | —         | 908                         |
| 2         | 28.5         | —           | —         | 720                         |
| 3         | 32.5         | —           | —         | 623                         |
| 4         | 24.8         | —           | 1.08      | 690                         |
| 5         | 24.5         | —           | 2.13      | 662                         |
| 6         | 22.8         | 0.99        | —         | 738                         |
| 7         | 21.3         | 0.93        | 0.93      | 661                         |
| 8         | 21.8         | 0.95        | 1.90      | 629                         |

The first three conditions span a range of starch dose within which the conditions containing the NCC, the copolymer and the blends are dosed. After accounting for the strengthening effect of starch, the abrasion loss results demonstrate that the NCC and the AA/AM copolymer have a similar level of performance. The effect is further enhanced when the additives are blended in a 50:50 and a 33:67 NCC:AA/AM ratio.

Next, a study was designed to determine whether growing an AA/AM copolymer on to the surface of the NCC improves the paper surface strength and compare its performance with that of the NCC. As part of this study, three NCC-Polymers varying in the AA/AM monomer ratio were tested. The table below shows the conditions and the results:

TABLE 6

| Condition | AA/AM monomer ratio | Starch, lb/t | NCC, lb/t | NCC-Polymer, lb/t | Abrasion loss, mg/1000 revs |
|-----------|---------------------|--------------|-----------|-------------------|-----------------------------|
| 1         | —                   | 17.5         | —         | —                 | 899                         |
| 2         | —                   | 23.1         | —         | —                 | 681                         |
| 3         | —                   | 27.2         | —         | —                 | 558                         |
| 4         | —                   | 22.9         | 1.00      | —                 | 640                         |
| 5         | 30/70               | 20.3         | —         | 0.88              | 631                         |
| 6         | 50/50               | 20.6         | —         | 0.90              | 598                         |
| 7         | 70/30               | 20.2         | —         | 0.88              | 633                         |

The first three conditions span a range of starch dose within which the conditions containing the NCC and NCC-Polymers are dosed. After accounting for the starch dose in each of the conditions, the abrasion loss results demonstrate that the grafting of the AA/AM copolymer on to the surface of the NCC is an improvement over the NCC. The surface strength performance is not affected, however, by the AA/AM monomer ratio in the 30/70 to 70/30 range.

Next, a study was designed to simultaneously compare surface strength performance as a function of all of the conditions (i.e., unmodified, modified with an anionic polymer of different mole ratios, and blends of the unmodified NCC with the AA/AM copolymer). The table below shows the conditions and the results.

TABLE 7

| Condition | Starch, lb/t | AA/AM, lb/t | NCC, lb/t | NCC-Polymer (30/70 AA/AM), lb/t | Abrasion loss, mg/1000 revs |
|-----------|--------------|-------------|-----------|---------------------------------|-----------------------------|
| 1         | 15.3         | —           | —         | —                               | 799                         |
| 2         | 27.2         | —           | —         | —                               | 507                         |
| 3         | 13.7         | 0.91        | —         | —                               | 772                         |
| 4         | 25.9         | 0.86        | —         | —                               | 451                         |

TABLE 7-continued

| Condition | Starch, lb/t | AA/AM, lb/t | NCC, lb/t | NCC-Polymer (30/70 AA/AM), lb/t | Abrasion loss, mg/1000 revs |
|-----------|--------------|-------------|-----------|---------------------------------|-----------------------------|
| 5         | 13.0         | 2.59        | —         | —                               | 644                         |
| 6         | 23.0         | 2.30        | —         | —                               | 399                         |
| 7         | 15.6         | —           | 1.04      | —                               | 725                         |
| 8         | 28.9         | —           | 0.96      | —                               | 505                         |
| 9         | 14.9         | —           | 2.98      | —                               | 725                         |
| 10        | 24.4         | —           | 2.44      | —                               | 422                         |
| 11        | 13.6         | —           | —         | 0.91                            | 761                         |
| 12        | 25.1         | —           | —         | 1.01                            | 443                         |
| 13        | 12.7         | —           | —         | 2.53                            | 708                         |
| 14        | 25.9         | —           | —         | 2.59                            | 401                         |
| 15        | 14.4         | 0.86        | 0.10      | —                               | 740                         |
| 16        | 22.3         | 0.67        | 0.07      | —                               | 441                         |
| 17        | 13.0         | 2.34        | 0.26      | —                               | 665                         |
| 18        | 22.2         | 2.00        | 0.22      | —                               | 382                         |

The first two conditions only contained starch, while the others contained about 1 or 3 lb/t of the additive. On conditions 15-18, the unmodified NCC:AAAM blends were prepared in a 10:90 mass ratio. The contributions of the multiple variables in this study were better elucidated with a regression analysis of the results. The model for the analysis resulted in a correlation coefficient of 0.80 with all variables (starch, the AA/AM copolymer, NCC, NCC-Polymer, and the blends of AA/AM copolymer and the NCC) statistically contributing to the model. From highest to lowest, the magnitude of their contribution to strengthening the paper surface is the following:

1. Blends of AA/AM copolymer and NCC
2. AA/AM copolymer
3. NCC-Polymer
4. NCC

While this invention may be embodied in many different forms, there are described in detail herein specific preferred embodiments of the invention. The present disclosure is an exemplification of the principles of the invention and is not intended to limit the invention to the particular embodiments illustrated. All patents, patent applications, scientific papers, and any other referenced materials mentioned herein are incorporated by reference in their entirety. Furthermore, the invention encompasses any possible combination of some or all of the various embodiments mentioned herein, described herein and/or incorporated herein. In addition the invention encompasses any possible combination that also specifically excludes any one or some of the various embodiments mentioned herein, described herein and/or incorporated herein.

The above disclosure is intended to be illustrative and not exhaustive. This description will suggest many variations and alternatives to one of ordinary skill in this art. All these alternatives and variations are intended to be included within the scope of the claims where the term "comprising" means "including, but not limited to". Those familiar with the art may recognize other equivalents to the specific embodiments described herein which equivalents are also intended to be encompassed by the claims.

All ranges and parameters disclosed herein are understood to encompass any and all subranges subsumed therein, and every number between the endpoints. For example, a stated range of "1 to 10" should be considered to include any and all subranges between (and inclusive of) the minimum value of 1 and the maximum value of 10; that is, all subranges beginning with a minimum value of 1 or more, (e.g. 1 to 6.1), and ending with a maximum value of 10 or less, (e.g. 2.3 to 9.4, 3 to 8, 4

## 15

to 7), and finally to each number 1, 2, 3, 4, 5, 6, 7, 8, 9, and 10 contained within the range. All percentages, ratios and proportions herein are by weight unless otherwise specified.

This completes the description of the preferred and alternate embodiments of the invention. Those skilled in the art may recognize other equivalents to the specific embodiment described herein which equivalents are intended to be encompassed by the claims attached hereto.

The invention claimed is:

1. A method of improving a paper substrate used in a papermaking process, the method comprising the steps of: adding an NCC-polymer to a paper substrate in the wet end of a papermaking process, wherein the NCC-polymer is substantially distributed throughout the paper substrate, wherein the NCC-polymer comprises an NCC-Core having a crystalline fraction of no less than 80%, and wherein the NCC-polymer is added in an amount less than or equal to 2.0 lb/ton of paper substrate.
2. The method of claim 1 wherein the NCC-polymer comprises a polymer chain bonded to an NCC core and the polymer chain is made up of one or more monomers selected from the list consisting of: vinyl acetate, acrylic acid, sodium acrylate, ammonium acrylate, methyl acrylate, acrylamide, acrylonitrile, N,N-dimethyl acrylamide, 2-acrylamido-2-methylpropane-1-sulfonic acid, sodium 2-acrylamido-2-methylpropane-1-sulfonate, 3-acrylamidopropyl-trimethylammonium chloride, diallyldimethylammonium chloride, 2-(dimethylamino)ethyl acrylate, 2-(acryloyloxy)-N,N,N-trimethyllethanaminium chloride, N,N-dimethylaminoethyl acrylate benzyl chloride quaternary salt, 2-(acryloyloxy)-N,N,N-trimethyllethanaminium methyl sulfate, 2-(dimethylamino)ethyl methacrylate, 2-(methacryloyloxy)-N,N,N-trimethyllethanaminium chloride, 3-(dimethylamino)propyl methacrylamide, 2-(methacryloyloxy)-N,N,N-trimethyllethanaminium methyl sulfate, methacrylic acid, methacrylic anhydride, methyl methacrylate, methacryloyloxy ethyl trimethyl ammonium chloride, 3-methacrylamidopropyl-trimethylammonium chloride, hexadecyl methacrylate, octadecyl methacrylate, docosyl acrylate, n-vinyl pyrrolidone, 2-vinyl pyridine, 4-vinyl pyridine, epichlorohydrin, n-vinyl formamide, n-vinyl acetamide, 2-hydroxyethyl acrylate glycidyl methacrylate, 3-(allyloxy)-2-hydroxypropane-1-sulfonate, 2-(allyloxy)ethanol, ethylene oxide, propylene oxide, 2,3-epoxypropyltrimethylammonium chloride, (3-glycidoxypropyl)trimethoxy silane, epichlorohydrin-dimethylamine, vinyl sulfonic acid
3. The method of claim 1 wherein the NCC-polymer is a graft polymer having at least two NCC cores linked at least in part by polymer chains.
4. The method of claim 1 wherein the NCC-polymer is a branched polymer having a first polymer chain extending from an NCC core and at least one branch diverting away from the first polymer chain.
5. The method of claim 4 wherein at least one branch is constructed out of a different selection of monomers than the first polymer chain, the different selection being different in monomer type, monomer ratio, or both.
6. The method of claim 1 wherein the NCC-polymer increases the wet strength of the paper substrate.
7. The method of claim 1 wherein the NCC-polymer increases the retention of solids during the drainage of liquid medium from the paper substrate.
8. The method of claim 1 wherein the NCC-polymer increases the dry strength of the paper substrate.
9. The method of claim 1 wherein the NCC-polymer increases the wet web strength of the paper substrate.
10. A method of improving a paper substrate used in a papermaking process, the method comprising the steps of: adding a blend to a paper substrate in the wet end of a papermaking process, wherein the blend comprises NCC mixed with a polymer and is substantially distributed throughout the paper substrate, wherein the NCC-polymer comprises an NCC-Core having a crystalline fraction of no less than 80%, and wherein the NCC-polymer is added in an amount less than or equal to 2.0 lb/ton of paper substrate.
11. A method of improving a paper substrate used in a papermaking process, the method comprising the steps of: adding an NCC-polymer to a paper substrate in the wet end of a papermaking process, wherein the NCC-polymer is substantially distributed throughout the paper substrate, wherein the NCC-polymer is a branched polymer having a first polymer chain extending from an NCC core and at least one branch diverting away from the first polymer chain, and wherein the NCC-polymer is added in an amount less than or equal to 2.0 lb/ton of paper substrate.
12. The method of claim 11 wherein at least one branch is constructed out of a different selection of monomers than the first polymer chain, the different selection being different in monomer type, monomer ratio, or both.

## 16

sodium salt, sodium 4-styrene sulfonate, caprolactam and any combination thereof.

5

3. The method of claim 1 wherein the NCC-polymer is a graft polymer having at least two NCC cores linked at least in part by polymer chains.

4. The method of claim 1 wherein the NCC-polymer is a branched polymer having a first polymer chain extending from an NCC core and at least one branch diverting away from the first polymer chain.

5. The method of claim 4 wherein at least one branch is constructed out of a different selection of monomers than the first polymer chain, the different selection being different in monomer type, monomer ratio, or both.

15 6. The method of claim 1 wherein the NCC-polymer increases the wet strength of the paper substrate.

7. The method of claim 1 wherein the NCC-polymer increases the retention of solids during the drainage of liquid medium from the paper substrate.

20 8. The method of claim 1 wherein the NCC-polymer increases the dry strength of the paper substrate.

9. The method of claim 1 wherein the NCC-polymer increases the wet web strength of the paper substrate.

25 10. A method of improving a paper substrate used in a papermaking process, the method comprising the steps of:

30 adding a blend to a paper substrate in the wet end of a papermaking process, wherein the blend comprises NCC mixed with a polymer and is substantially distributed throughout the paper substrate, wherein the NCC-polymer comprises an NCC-Core having a crystalline fraction of no less than 80%, and wherein the NCC-polymer is added in an amount less than or equal to 2.0 lb/ton of paper substrate.

35 11. A method of improving a paper substrate used in a papermaking process, the method comprising the steps of:

30 adding an NCC-polymer to a paper substrate in the wet end of a papermaking process, wherein the NCC-polymer is substantially distributed throughout the paper substrate, wherein the NCC-polymer is a branched polymer having a first polymer chain extending from an NCC core and at least one branch diverting away from the first polymer chain, and wherein the NCC-polymer is added in an amount less than or equal to 2.0 lb/ton of paper substrate.

40 45 12. The method of claim 11 wherein at least one branch is constructed out of a different selection of monomers than the first polymer chain, the different selection being different in monomer type, monomer ratio, or both.

\* \* \* \* \*